

Patented Aug. 7, 1945

2,381,049

# UNITED STATES PATENT OFFICE

2,381,049

## PRESERVATION AND FIREPROOFING OF WOOD

Richard Newton Hammond, Longview, Wash., as-  
signor to General Timber Service, Inc., St. Paul,  
Minn., a corporation of Delaware

No Drawing. Application March 18, 1939.  
Serial No. 262,666

6 Claims. (Cl. 117—59)

This invention relates to the preservation and fireproofing of wood and particularly to an improved method of introducing toxic or fireproofing materials into wood to increase its resistance to the attack of fungi and other wood-destroying organisms or to make the wood resistant to fire. Either or both of these objects may be accomplished by the procedure hereinafter more fully described.

Wood consists of groups of cells, the walls of which are principally of cellulose. When wet, cellulose acts as a semi-permeable membrane allowing the passage of substances in true water solution, and preventing the passage of colloids. A cellulose membrane separating water from a water solution will allow free passage of solvent and solute molecules through the cellulose lattice until the concentration of the solute is the same on both sides of the membrane. If, however, there is substantially no water on one side of the membrane, the movement of solvent and solute practically ceases. Hence it is impracticable to impregnate wood with water solutions satisfactorily when the wood is dry or substantially dry, unless auxiliary means are employed. Materials which are not water solutions do not penetrate the cell walls and can be introduced into the wood only through the pits, cracks and checks which exist therein, and can be introduced through the side grain only by the application of pressure. Consequently, the methods of impregnating wood heretofore have depended primarily upon procedures involving the application of pressure to the impregnating material, either with or without initial treatment to evacuate, so far as possible, the contents of the cells so that the impregnating material can be forced mechanically into the wood. At best only a limited impregnation of many woods can be secured by the methods heretofore used.

It is the object of the present invention to afford a more satisfactory and practicable method of impregnating wood with various solutions adapted, because of their toxic nature, to retard the development of wood-destroying organisms, or to make the wood fire-resistant, or for both of these purposes.

Another object of the invention is the provision of a method whereby various solutions may be introduced effectively into the wood cells without the necessity for applying external pressure.

Other objects and advantages of the invention will be apparent as it is better understood by reference to the following specification, in which preferred embodiments of the invention are described, it being understood that the examples are merely illustrative of a wide variety of solutions and substances which can be utilized in accordance with the method to accomplish the purposes mentioned.

The heartwood of the various woods used for construction purposes, and therefore those which are treated to prevent destruction by fungi and other wood-destroying organisms, contains only 5 slightly more than enough moisture to saturate the wood fibres. Solutions containing toxic materials or materials adapted to make the wood fire-resistant, will not penetrate the cell walls of the wood to any appreciable extent by diffusion. 10 I have discovered, however, that if the wood is first treated to increase the moisture content of the cells, the rate of diffusion of solutions containing toxic and other materials increases rapidly, and consequently it is possible without the aid of mechanical pressure, to thoroughly impregnate the wood with the desired solutions in a relatively brief time.

Accordingly, I subject the wood, prior to its treatment with the desired solution, to an initial 20 treatment by soaking it in hot water for a sufficient length of time to effect the desired increase in the moisture content of the wood cells. The temperature at which the initial treatment is conducted may vary over a wide range. Since 25 temperatures below 120° F. cannot be considered effective in killing fungus growth already present in the wood, I consider this the lower limit. Temperatures up to 212° F. or higher may be used. In the latter case, the steam or vapor 30 should be of 100% relative humidity.

The length of time required for the water treatment depends upon the size of the material to be treated and would be from two hours for very thin stock to approximately two days for very 35 thick material. Necessarily the time is adjusted in accordance with experience based upon the treatment of materials in varying sizes.

When the wood has been subjected for a sufficient time to the effect of the hot water, so that 40 the wood cells contain a sufficient quantity of water, the wood is immediately subjected to immersion in a suitable solution containing the material with which the wood is to be impregnated. The time of immersion will vary as in the initial 45 treatment, depending upon the thickness of the wood. From one to ten days may be required, depending also on the concentration of the chemicals in the treating solution, the desired quantitative absorption of toxic and fireproofing agents, 50 and the depth of chemical penetration desired.

A large variety of materials may be used for the treatment of wood in accordance with the invention, and the treatment may be in one or two stages, depending upon the character of the 55 materials used. Thus, it is possible to select a chemical agent which may be toxic to wood-destroying organisms or capable of rendering the wood resistant to fire. Numerous agents of this type are known, and the immersion of the wood 60 in a solution of one of these materials for a suf-

ficient length of time will serve to impregnate the wood and accomplish the desired result. In some cases, however, either the preservative or the fire-proofing effect may be accomplished by immersing the wood in two different solutions successively, so that the solutions will react within the wood cells to deposit a compound having the desired effect. In some cases, both the preservative and fireproofing effects can be secured by the selection of suitable materials. In some cases, a third step may be introduced, involving the application of a reactive gas to the wood.

The two-stage treatment has the advantage that whereas water soluble solutions with which the wood may be impregnated may be leached therefrom when the wood is in contact with water, wet soil, etc., the formation of insoluble compounds within the wood cells ensures the retention of the toxic or fireproofing agent regardless of the presence of water. The two-stage operation for depositing insoluble compounds has been described heretofore in connection with impregnation processes depending upon pressure, but in such cases the pores and checks in the wood are quickly plugged by precipitation of the insoluble material, and very shallow penetration is secured. By the present method the introduction of the insoluble compounds to the cells of the wood is assured because reaction does not occur until the two solutions meet within the cells.

The following examples will illustrate the application of the invention in respect to types of solutions which may be used to impregnate the wood, following the initial treatment with hot water. The invention is not limited to the particular compounds mentioned, since as already indicated it depends upon the initial treatment with hot water to increase the moisture content of the cells so that diffusion through the walls thereof is made possible or accelerated. Furthermore, the temperatures, time of treatment and concentration of the solutions, are subject to wide variation, depending, as already noted, on a number of factors which must be considered in the practical application of the method.

is the reduction in the cost of equipment as contrasted with processes employing pressure, which require closed containers adapted to withstand the pressure. A further advantage is efficiency with respect to the degree of impregnation, since it depends upon diffusion. The efficiency of pressure in introducing solutions or materials into the wood is relatively low, whereas diffusion ensures the introduction of the materials into the wood cells. Another advantage is the degree of control which can be employed by varying the factors such as time, temperature and concentration of the solutions used. Such control is not readily effected with pressure processes.

Various changes may be made in the procedure without departing from the invention or sacrificing the advantages thereof.

I claim:

1. The method of impregnating wood which comprises treating the wood with liquid water at a temperature above about 120° F. for a length of time sufficient to increase substantially the moisture content of the wood cells, and, while the moisture content of the wood cells is substantially increased, immersing the wood in a water solution

20 of the material with which the wood is to be impregnated, and permitting the water solution of the impregnating material to diffuse into the cells of the wood.

25 2. The method of impregnating wood which comprises treating the wood at atmospheric pressure with liquid water at a temperature between about 120° F. and 212° F. for a length of time sufficient to increase substantially the moisture content of the cells thereof, and, while the moisture content of the wood is substantially increased, immersing the wood in two successive aqueous solutions, the compositions of which are such that they react to form a precipitate, and permitting each of said successive solutions to diffuse into the cells of the wood where they react to form a precipitate.

30 3. The method of impregnating wood which comprises treating the wood with liquid water at a temperature above about 120° F. for a length of time sufficient to increase substantially the moisture content of the wood cells, and, while the moisture content of the wood is substantially increased, immersing the wood in two successive aqueous solutions, the compositions of which are such that they react to form a precipitate, and permitting each of said successive solutions to diffuse into the cells of the wood where they react to form a precipitate.

35 4. The method of impregnating wood which comprises treating the wood with liquid water at a temperature above about 120° F. for a length of time sufficient to increase substantially the moisture content of the wood cells, and, while the moisture content of the wood is substantially increased, immersing the wood in two successive aqueous solutions, the compositions of which are such that they react to form a precipitate, and permitting each of said successive solutions to diffuse into the cells of the wood where they react to form a precipitate.

40 5. The method of impregnating wood which comprises treating the wood with liquid water at a temperature above about 120° F. for a length of time sufficient to increase substantially the moisture content of the wood cells, and, while the moisture content of the wood is substantially increased, immersing the wood in two successive aqueous solutions, the compositions of which are such that they react to form a precipitate, and permitting each of said successive solutions to diffuse into the cells of the wood where they react to form a precipitate.

45 6. The method of impregnating wood which comprises treating the wood with liquid water at a temperature above about 120° F. for a length of time sufficient to increase substantially the moisture content of the wood cells, and, while the moisture content of the wood is substantially increased, immersing the wood in two successive aqueous solutions, the compositions of which are such that they react to form a precipitate, and permitting each of said successive solutions to diffuse into the cells of the wood where they react to form a precipitate.

| Type material                                                            | Preliminary treatment                        | Time preliminary treatment | Toxic solution and concentration                                | Time in toxic solution | Temperature treatment solution |
|--------------------------------------------------------------------------|----------------------------------------------|----------------------------|-----------------------------------------------------------------|------------------------|--------------------------------|
| <b>EXAMPLES OF WOOD PRESERVING TREATMENTS</b>                            |                                              |                            |                                                                 |                        |                                |
| Douglas fir 2" x 12" x 18'<br>W. hemlock 2" x 2" x 5'                    | Water 120° to (hot) 100°<br>Water 212° (hot) | Hours<br>24<br>18          | 12.5% chromated zinc chloride<br>18.7% zinc chloride            | Hours<br>72<br>48      | °F.<br>50<br>80                |
| <b>EXAMPLE OF FIREPROOFING TREATMENT</b>                                 |                                              |                            |                                                                 |                        |                                |
| Vertical grain D. fir flooring                                           | Water 120° F. (hot)                          | 12                         | 20% monoammonium phosphate                                      | 48                     | 60                             |
| <b>EXAMPLE OF COMBINATION FIREPROOFING AND PRESERVING TREATMENTS</b>     |                                              |                            |                                                                 |                        |                                |
| Douglas fir 2" x 12" x 6'                                                | Water 200° F. (hot)                          | 18                         | 12.5% zinc chloride-15% monoammonium phosphate                  | 48                     | 60                             |
| <b>EXAMPLE OF 2-STAGE TREATMENT FOR BOTH FIREPROOFING AND PRESERVING</b> |                                              |                            |                                                                 |                        |                                |
| Douglas fir 2" x 12" x 6'                                                | Water 200° F. (hot)                          | 18                         | #1-12% chromated zinc chloride<br>#2-15% monoammonium phosphate | 48                     | 60                             |

Alternative step #3 followed by treatment in ammonia gas.<sup>1</sup>

<sup>1</sup> This wood after drying contains zinc chromate, zinc ammonium phosphate, ammonium phosphate and ammonium chloride.

The method as herein described has numerous advantages, among the most important of which

moisture content of the wood cells, immersing the wood in a water solution of zinc chloride

while the moisture content of the cells thereof is substantially increased, and permitting said water solution to diffuse into the cells of the wood.

4. The method of impregnating wood which comprises treating the wood with liquid water at a temperature above about 120° F. for a length of time sufficient to increase substantially the moisture content of the wood cells, immersing the wood in a water solution of chromated zinc chloride while the moisture content of the cells thereof is substantially increased, and permitting said water solution to diffuse into the cells of the wood.

5. The method of impregnating wood which comprises treating the wood with liquid water at a temperature above about 120° F. for a length of time sufficient to increase substantially the moisture content of the wood cells, immersing the wood in a water solution of mono-ammonium

phosphate while the moisture content of the cells thereof is substantially increased, and permitting said water solution to diffuse into the cells of the wood.

6. The method of impregnating wood which comprises treating the wood at atmospheric pressure with liquid water at a temperature between about 120° F. and 212° F. for a length of time sufficient to increase substantially the moisture content of the cells thereof, immersing the wood successively in aqueous solutions of chromated zinc chloride and mono-ammonium phosphate while the moisture content of the cells thereof is substantially increased, and permitting the wood to remain in each of said aqueous solutions for a length of time sufficient for them to diffuse into the cells of the wood, whereby a precipitate is formed in the cells of the wood.

RICHARD NEWTON HAMMOND.